

# United States Patent

Hayakawa et al.

[15] 3,656,961

[45] Apr. 18, 1972

[54] **DIRECT POSITIVE SILVER HALIDE PHOTOGRAPHIC LIGHT-SENSITIVE ELEMENTS**

[72] Inventors: Yoshihide Hayakawa, Saitama; Hideo Kawano, Kanagawa; Hirotetu Kato, Kanagawa, all of Japan

[73] Assignee: Fuji Photo Film Co., Ltd., Kanagawa, Japan

[22] Filed: Jan. 7, 1970

[21] Appl. No.: 1,302

[30] **Foreign Application Priority Data**

Jan. 25, 1969 Japan..... 44/5582

[52] U.S. Cl..... 96/108, 96/107

[51] Int. Cl..... G03c 1/28

[58] Field of Search..... 96/107, 64, 108

[56]

**References Cited**

**UNITED STATES PATENTS**

|           |        |                |       |
|-----------|--------|----------------|-------|
| 2,717,833 | 9/1955 | Work.....      | 96/64 |
| 3,035,917 | 5/1962 | Fry et al..... | 96/64 |

Primary Examiner—Norman G. Torchin

Assistant Examiner—Richard E. Fichter

Attorney—Sughrue, Rothwell, Mion, Zinn & Macpeak

[57]

**ABSTRACT**

A light-sensitive, direct positive, photographic silver halide element comprising a support having thereon a silver halide emulsion layer containing a salt selected from the group consisting of a soluble salt and a complex salt of a metal belonging to Group 8 of the periodic table and a condensed polycyclic quinone compound.

14 Claims, No Drawings

# DIRECT POSITIVE SILVER HALIDE PHOTOGRAPHIC LIGHT-SENSITIVE ELEMENTS

## BACKGROUND OF THE INVENTION

### 1. Field of the Invention

The present invention relates to a direct positive photographic silver halide element. More particularly, it relates to a light-sensitive, direct positive, photographic silver halide element capable of providing direct positive images having low residual minimum density, a wide exposure latitude and a high contrast by only one exposure and one development.

### 2. Description of the Prior Art

A light-sensitive, direct positive, photographic silver halide element is a photographic element wherein, as the amount of exposure applied to the element increases, the optical density of the image formed thereon after development is reduced. It is well known that by adding a desensitizing agent to the photographic silver halide emulsion during the preparation of the photographic light-sensitive element, the reversal sensitivity speed is markedly increased.

As the aforesaid desensitizing agents, there are known such organic compounds as pinakryptol yellow and pinakryptol green, and compounds which contain a metal of Group 8 of the Periodic Table, such as rhodium and iridium compounds (see, e.g., U.S. Pat. No. 2,717,833).

However, in conventional light-sensitive, direct positive, photographic silver halide elements inwhich the aforesaid known desensitizing agents are utilized, an effect known as the Herschel effect occurs, and hence the sensitivity is low. It is also necessary to expose the light-sensitive element to light through a yellow filter. That is, if a yellow filter is not used during the exposure of the light-sensitive element, no positive images are obtained or, if any positive images are obtained, they are inferior in quality. In this case, the above-mentioned occurrence of the inferior image quality is caused by the fact that a negative image is formed by a so-called re-reversal phenomenon, that is, a phenomenon wherein as the amount of exposure increases, the optical density of the formed images after development is increased again over the minimum value and the negative image thus formed is superposed on the positive image.

Therefore, an object of the present invention is to provide a light-sensitive, direct positive, photographic silver halide element having a wide exposure latitude and being capable of providing hard direct positive images having high contrast.

## SUMMARY OF THE INVENTION

According to the present invention, a salt of a metal belonging to Group 8 of the periodic table and a condensed polycyclic quinone are incorporated into the photographic light-sensitive emulsion.

## DETAILED DESCRIPTION OF THE PREFERRED EMBODIMENTS

The metals belonging to Group 8 of the periodic table which may be employed in the present invention include rhodium, iridium, ruthenium, palladium, osmium, cobalt, and platinum. The metals may be employed in the form of water-soluble salts, such as, halides and nitrates of these metals or as complex salts thereof, in particular, as complex salts having the formula,



wherein A represents an alkali metal or a hydrogen atom, M represents the Group 8 metal, and X represents a halogen atom.

As the condensed polycyclic quinones to be employed in the present invention, there may be illustrated the following: naphthoquinone, anthraquinone, phenanthraquinone, and derivatives thereof. The following are particularly preferable: sodium anthraquinone-2,6-disulfonate,  $\alpha$ -naphthoquinone, 2-chloroanthraquinone, sodium anthraquinone- $\beta$ -sulfonate, 1,5-dichloroanthraquinone, and 1,2-benzanthraquinone.

The photographic silver halide emulsion to which the aforesaid compounds are added consists of a protective colloid such as gelatin or a hydrophilic organic colloid having dispersed therein silver chloride, silver chlorobromide, silver bromide, silver iodobromide, silver chlorobromide, or silver chloroiodobromide.

The above-mentioned salt of the Group 8 metal is incorporated in the aforesaid silver halide photographic emulsion during the emulsification of the silver halide or during physical ripening of the photographic emulsion. The preferable amount of the metal salt to be added is from  $1 \times 10^{-6}$  mole to  $1 \times 10^{-2}$  mole, particularly from  $1 \times 10^{-4}$  mole to  $1 \times 10^{-3}$  mole, per 1 mole of silver halide.

The amount of the condensed polycyclic quinone to be used with the above-mentioned metal salt depends upon the nature of the polycyclic quinone and silver halide emulsion to be employed but is preferably from 5 mg. to 500 mg. per 1 mole of silver halide. The condensed polycyclic quinone may be added in the silver halide emulsion at any stage but is most preferably added thereto at a stage after the completion of the formation of fogged nuclei and before coating. The condensed polycyclic quinone may be added to the photographic silver halide emulsion while dissolved in a solvent that has no deleterious effect on the emulsion, such as water, a lower alcohol having from one to five carbon atoms, or a ketone.

In the present invention, better results may be obtained by using, together with the two ingredients mentioned above, a known desensitizing agent such as pinakryptol yellow, pinakryptol green, or phenoxyfranine. This third ingredient is preferably added to the silver halide emulsion just before coating.

The direct reversal silver halide photographic light-sensitive element of the present invention may be prepared in the following manner. A silver halide emulsion is prepared according to a conventional method of precipitation and physical ripening, forming fogged nuclei in the silver halide emulsion by exposing or by alkalinizing the silver halide emulsion and adding thereto a reducing agent such as formaldehyde, hydrazine, a divalent tin salt, thiourea dioxide, or an amine compound. Thereafter, the emulsion is applied to a suitable support, after adding thereto the aforesaid metal salt and the condensed polycyclic quinone together with, if necessary, the above-mentioned desensitizing agent. The support may be a cellulose acetate film, a polyethylene terephthalate film, a baryta-coated paper, a synthetic paper, or a waterproof paper. Then, the assembly is dried. Moreover, ordinary photographic additives such as hardening agents, surface active agents, and sensitizing dyes may be added to the silver halide emulsion.

As will be shown in the following examples the light-sensitive direct positive, photographic silver halide element of the present invention has an excellent exposure latitude and provides a direct positive image having a high contrast.

The present invention will be further illustrated by reference to the following examples.

## EXAMPLE 1

To a 10 percent aqueous gelatin solution were added simultaneously an aqueous solution containing 100 g. of silver nitrate and an aqueous solution containing 30 g. of sodium chloride, 20 g. of potassium bromide and 10 mg. of rhodium chloride to form fine silver halide particles. Thereafter, 1 g. of potassium iodide and 40 g. of gelatin were added to the silver halide emulsion and then the pH of the emulsion was adjusted to 9.5 with sodium carbonate. Then, 3 ml. of a 1 percent aqueous hydrazine chloride solution was added to the emulsion and the resultant emulsion was ripened for 40 minutes to form fogged nuclei. After ripening, the pH of the silver halide emulsion was adjusted to 6.0 with a 10 percent aqueous citric acid solution. The resultant silver halide emulsion was cooled, washed with water, and sodium anthraquinone-2,6-disulfonate together with pinakryptol yellow in the amounts shown in Table 1 were added to the emulsion. As a control example,

photographic silver halide emulsions were prepared in a similar manner as above except that no rhodium salt was added.

TABLE 1

| Emulsion No. | Rhodium chloride | Concentration* of Ingredients | Pinakryptol yellow |
|--------------|------------------|-------------------------------|--------------------|
| 1            | 0                | 0                             | 100                |
| 2            | 0                | 200                           | 0                  |
| 3            | 0                | 100                           | 50                 |
| 4            | 10               | 0                             | 0                  |
| 5            | 10               | 0                             | 100                |
| 6            | 10               | 200                           | 0                  |
| 7            | 10               | 100                           | 50                 |

\*(note): the unit of concentration is mg./l mole of Ag.

Each of the photographic silver halide emulsions prepared above was coated on a cellulose triacetate film and dried.

The light sensitive, direct positive, photographic films prepared above were exposed through an optical wedge to a tungsten lamp of 2,660° K. and developed for 3 minutes at 20° C. in a developer having the following composition:

|                            |           |
|----------------------------|-----------|
| Water                      | 500 ml.   |
| Sodium sulfite (anhydrous) | 30 g.     |
| Paraformaldehyde           | 7.5 g.    |
| Borax                      | 7.5 g.    |
| Sodium bisulfite           | 2.2 g.    |
| Hydroquinone               | 22.5 g.   |
| Potassium bromide          | 1.6 g.    |
| Water to make              | 1,000 ml. |

The minimum density, the contrast, and the exposure latitude of the samples prepared are shown in Table 2.

TABLE 2

| Test No. | Minimum density | Contrast | Exposure latitude |
|----------|-----------------|----------|-------------------|
| 1        | 0.09            | 2.4      | 0.9               |
| 2        | 0.09            | 2.3      | 0.9               |
| 3        | 0.09            | 2.5      | 1.0               |
| 4        | 0.10            | 2.4      | 0.9               |
| 5        | 0.07            | 2.4      | 2.0               |
| 6        | 0.05            | 4.8      | 3.1               |
| 7        | 0.05            | 4.6      | 3.1               |

The contrast shown in the above table is the mean gradient between point 1 (base density of characteristic curve + fog density + density 0.1) and point 2 (base density of characteristic curve + fog density + density 2.1).

The exposure latitude in the above table is shown by the difference ( $\log E_2 - \log E_1$ ) between logarithms of the exposure amount  $\log E_2$  giving (base density + fog density + density 2.1) of the negative image portion, and the exposure amount  $\log E_1$  giving (base density + fog density + density 2.1) of the positive image portion.

From the results shown in Table 2, it is readily apparent that samples 6 and 7 had much wider exposure latitudes, higher contrast and lower minimum density than the other samples.

## EXAMPLE 2

To a 10 percent aqueous gelatin solution were added, simultaneously, an aqueous solution containing 100 g. of silver nitrate and an aqueous solution containing 30 g. of sodium chloride, 20 g. of potassium bromide, and 10 mg. of iridium chloride, to thereby form fine silver halide particles. Thereafter, 1 g. of potassium iodide and 40 g. of gelatin were added to the silver halide emulsion and the pH of the resultant emulsion was adjusted to 9.5 with sodium carbonate.

After adding 5 ml. of a 0.1 percent aqueous thiourea dioxide solution, the emulsion was ripened for 40 minutes to form fogged nuclei and then the pH of the emulsion was adjusted to 6.0. After cooling and washing with water, 2-chloroanthraquinone and pinakryptol yellow were added to the emulsion as shown in Table 3. Also, as control samples,

similar silver halide emulsions containing no iridium chloride were prepared by a method similar to the above method.

Each of the photographic silver halide emulsions thus prepared was coated on a polyethylene terephthalate film and dried. The light-sensitive films thus prepared were exposed and developed as in Example 1. The results (the minimum density, contrast and the exposure latitude) are shown in Table 4.

TABLE 3 (mg./mole Ag)

| Emulsion No. | Iridium chloride | Concentration of Ingredients | Pinakryptol yellow |
|--------------|------------------|------------------------------|--------------------|
| 1            | 0                | 0                            | 100                |
| 2            | 0                | 200                          | 0                  |
| 3            | 0                | 100                          | 50                 |
| 4            | 20               | 0                            | 0                  |
| 5            | 20               | 0                            | 100                |
| 6            | 20               | 200                          | 0                  |
| 7            | 20               | 100                          | 50                 |

TABLE 4

| Test No. | Minimum density | Contrast | Exposure Latitude |
|----------|-----------------|----------|-------------------|
| 1        | 0.10            | 2.1      | 0.8               |
| 2        | 0.10            | 2.3      | 0.8               |
| 3        | 0.10            | 2.2      | 0.9               |
| 4        | 0.11            | 2.3      | 0.7               |
| 5        | 0.08            | 2.4      | 1.5               |
| 6        | 0.06            | 4.4      | 3.0               |
| 7        | 0.05            | 4.6      | 2.9               |

From the results shown in Table 4, it is apparent that samples 6 and 7 had an extremely wider exposure latitude, lower minimum densities and higher contrast than the other samples.

### 35 What is claimed is:

1. A light-sensitive, direct positive, photographic silver halide element comprising a support having thereon a silver halide emulsion layer containing a soluble nitrate, halide, or a complex salt of a metal selected from the group consisting of rhodium, iridium, ruthenium, palladium, osmium, cobalt and platinum, and a condensed polycyclic quinone compound.

2. The light-sensitive, direct positive, photographic silver halide element as in claim 1 wherein said complex salt is represented by the formula



wherein A represents an alkali metal or a hydrogen atom, M represents rhodium, iridium, ruthenium, palladium, osmium, cobalt or platinum, and X represents a halogen atom.

3. The light-sensitive, direct positive, photographic silver halide element as in claim 1 wherein said condensed polycyclic quinone is selected from the group consisting of sodium anthraquinone-2,6-disulfonate,  $\alpha$ -naphthoquinone, 2-chloroanthraquinone, sodium anthraquinone- $\beta$ -sulfonate, 1,5-dichloro-anthraquinone, and 1,2-benzanthraquinone.

4. The light-sensitive, direct positive, photographic silver halide element as in claim 1 wherein said salt is incorporated in said silver halide photographic emulsion during the emulsification or physical ripening of said silver halide emulsion and wherein said condensed polycyclic quinone is incorporated in said silver halide photographic emulsion at a stage after the completion of the formation of fogged nuclei and before the coating of said emulsion onto said support.

5. The light-sensitive, direct positive photographic silver halide element as in claim 1, wherein the amount of said salt in said emulsion layer is from  $10^{-6}$  mole to  $10^{-2}$  mole, per 1 mole of silver halide.

6. The light-sensitive, direct positive, photographic silver halide element as in claim 1, wherein the amount of said quinone compound in said emulsion layer is from 5 mg. to 500 mg., per 1 mole of silver halide.

7. A light-sensitive, direct positive photographic silver halide element comprising a support having thereon a silver halide emulsion layer containing

a soluble nitrate, halide, or a complex salt of a metal selected from the group consisting of rhodium, iridium, ruthenium, palladium, osmium, cobalt and platinum, a condensed polycyclic quinone, and a desensitizing agent.

8. A light-sensitive direct positive, photographic silver halide element as in claim 7 wherein said complex salt is represented by the formula



wherein A represents an alkali metal or a hydrogen atom, M represents rhodium, iridium, ruthenium, palladium, osmium, cobalt or platinum, and X represents a halogen atom.

9. The light-sensitive, direct positive, photographic silver halide element as in claim 7 wherein said condensed polycyclic quinone is selected from the group consisting of sodium anthraquinone,  $\alpha$ -naphthoquinone, 2-chloroanthraquinone, sodium anthraquinone- $\beta$ -sulfonate, 1,5-dichloroanthraquinone, and 1,2-benzanthraquinone.

10. The light-sensitive, direct positive, photographic silver halide element as claimed in claim 7 wherein said salt is incorporated in said silver halide emulsion during the emulsification or physical ripening of said silver halide emulsion and

wherein said condensed polycyclic quinone is added to said silver halide emulsion at a stage after the completion of the formation of fogged nuclei and before the coating of said emulsion onto said support.

11. The light-sensitive, direct positive photographic silver halide element as in claim 7 wherein said desensitizing agent is selected from the group consisting of pinakryptol yellow, pinakryptol green and phenoxyaniline.

12. The light-sensitive, direct positive, photographic silver halide element as in claim 7 wherein said desensitizing agent is incorporated in said silver halide emulsion just before the silver halide emulsion is applied to said support.

13. The light-sensitive, direct positive, photographic silver halide element as in claim 7, wherein the amount of said salt in said emulsion layer is from  $10^{-6}$  mole to  $10^{-2}$  mole, per 1 mole of silver halide.

14. The light-sensitive, direct positive, photographic silver halide element as in claim 7, wherein the amount of said quinone compound in said emulsion layer is from 5 mg. to 500 mg., per 1 mole of silver halide.

\* \* \* \* \*

25

30

35

40

45

50

55

60

65

70

75